

G. BATTY.  
APPARATUS FOR CASTING INGOTS.  
APPLICATION FILED MAY 11, 1920.

1,414,394.

Patented May 2, 1922.

3 SHEETS—SHEET 1.

Fig. 1.



Fig. 2.



Inventor:  
George Batty.  
Attorney: *W. H. Hailey*

1,414,394.

G. BATTY.  
APPARATUS FOR CASTING INGOTS.  
APPLICATION FILED MAY 11, 1920.

Patented May 2, 1922.

3 SHEETS—SHEET 2.

Fig. 3.



Fig. 4.



Inventor:  
George Batty.  
Attorney: W. H. Hadden.

1,414,394.

G. BATTY,  
APPARATUS FOR CASTING INGOTS,  
APPLICATION FILED MAY 14, 1920.

Patented May 2, 1922.

3 SHEETS—SHEET 3.

Fig. 5.



Fig. 7.



Fig. 6.



Fig. 8.



Fig. 10.



Fig. 9.



Fig. 11.



Fig. 12.



Fig. 13.

Inventor:  
George Batty  
Attorney: W.H. Alderman

# UNITED STATES PATENT OFFICE.

GEORGE BATTY, OF YORK, ENGLAND.

## APPARATUS FOR CASTING INGOTS.

1,414,394.

Specification of Letters Patent.

Patented May 2, 1922.

Application filed May 11, 1920. Serial No. 380,624.

To all whom it may concern:

Be it known that I, GEORGE BATTY, of York, England, a subject of the King of England, have invented certain new and useful Improvements in Apparatus for Casting Ingots, of which the following is a specification.

This invention relates to a novel method of casting ingots of steel and other metals.

10 In the usual method for the "cluster" casting of ingots with the use of a base plate and channelled runner-bricks, the base plate is recessed to receive the bricks and a central distribution-brick is used also having 15 channels communicating with those of the runner bricks, said base plates being designed for casting various numbers of ingots from a single central feeding trumpet located over the distributor-brick. In the operation of such method the moulds are 20 placed over holes in the runner bricks disposed centrally to the base of the moulds and the metal is discharged down the "trumpet" and thence through the distributor-brick 25 and runner-bricks into the moulds. This operation is known as "bottom casting" and is commonly practised where a large number of ingots are to be produced from one "cast."

The present invention however provides a 30 method in which certain disadvantages, hereinafter mentioned inherent to the operation of casting down a "trumpet" are eliminated, and accordingly instead of casting down the trumpet and through a distributor 35 brick and runner bricks as described above, the metal is cast down a mould placed centrally to a number of other moulds of equal cross sectional area, say four, eight or twelve of such moulds. The base plate differs in 40 design for each number of ingots required to be cast on each plate.

The invention also provides means for reducing the amount of ingot discarded due to "pipe" or "pocket" for which purpose I provide 45 refractory feeder heads or nozzles which are heated and placed in the outer moulds during the casting operation. The casting down the central mould continues until the metal reaches a certain level in the "nozzles" 50 the function of which is to maintain the metal in a fluid condition sufficiently long to avoid all "cavity" in the ingot due to contraction. The central mould may also be provided with such a nozzle which is inserted immediately 55 the "nozzles" of the outer moulds are fully charged.

In a modification of the method adapted for use with certain grades of steel the nozzles of the outer moulds are replaced by solid metal stoppers adapted to be held in a predetermined position in the moulds and with which the metal comes in contact during the casting operation causing the metal to freeze over and solidify at the surface. The casting in the central mould is continued at a reduced speed until the metal therein reaches a level higher than the "stoppered" surface of the ingots in the outer moulds a heated nozzle being then inserted in the central mould and filled with metal. The greater volume of metal in the central mould enables contraction cavities in the outer mould ingots to be eliminated and constitutes a means by which the outer ingots are fed under pressure from the central mould.

In order that the method may be applied to the production of large ingots I have also devised a special form of stopper which will yield better results than would be the case than if the solid metal stoppers above referred to were used. Such a stopper comprises a frame of cast steel or cast iron containing bricks of silica or other refractory material suitably recessed, the whole being carried by means such as a rod pierced with holes at different levels to admit of "stoppering off" the ingots at various desired lengths.

Embodiments of apparatus for carrying out the invention are illustrated in the accompanying drawings wherein:

Fig. 1 is a vertical section showing a base plate with a central and two outer moulds mounted thereon and "nozzles" or feeder heads applied to all the moulds.

Fig. 2 is a top plan view of base plate detached for the casting of nine ingots.

Fig. 3 is a view similar to Fig. 1 showing the stoppers above-mentioned applied to the outer moulds and

Fig. 4 is a detail sectional view of a special form of "nozzle."

Figs. 5 to 13 are various detail views of the composite metal and refractory stopper above referred to. Figs. 5 to 9 illustrating the metal frame and Figs. 10 to 13 the refractory bricks.

Taking as example an eight-way base plate *a* for producing nine ingots as illustrated in Fig. 2, eight channels *b* are formed in said base plate to receive the channelled runner-bricks *c*, said channels *b* communicating with the central recess *d* into which

is inserted a plate of steel *e* to prevent the erosion of the base plate by the hot metal. The said central plate *e* is cast of metal similar in composition to that of the ingot to be produced and is held in the recess by the runner-bricks *c* which all slightly overlap the aforesaid central recess as indicated at *f*.

The central mould *g* is mounted above the plate *e* and the outer moulds *h* each one 10 above the outer ends of the runner bricks *c* with which they communicate.

When in position as described the runner-bricks form an octagonal recess *d* the diameter of which must not be greater than 15 the diameter of the central or "feeder" mould *g* above referred to. The moulds are placed in position and the metal is cast down the feeder mould whence it flows through the runner bricks into each of the other moulds 20 this arrangement resulting in one ingot being top-cast, the metal entering from above and the remainder being bottom-cast as the metal enters at the base of the mould.

The means for reducing the amount of 25 "ingot" discarded due to "pipe" or "pocket" comprises refractory feeder heads or "dozzles" *i* of roughly rectangular section with a circular hole *j* and having enlarged upper outer diameter as at *i*<sup>1</sup> to produce a collar or 30 overhang *i*<sup>2</sup>. These dozzles are heated in any suitable furnace near the casting pit and are placed on the outer moulds *h* during the operation of casting. The lower part of the "dozzle" is inserted into the top of the mould 35 as indicated in Fig. 1 but is prevented from slipping down by the overhung portion *i*<sup>2</sup> and on each dozzle there may be placed a small weight such as of bar scrap, serving to prevent it from floating up when reached 40 by the metal. The casting down the central mould continues until the level of metal in the dozzles on outer moulds *h* reaches approximately the line *k* just below the enlarged or overhung portion and the function 45 of the "dozzles" is to maintain the metal in a fluid condition sufficiently long to obviate all "cavity" due to contraction. The central mould *g* may also be provided with a heated dozzle *l* which is inserted immediately after 50 the dozzles of the outer moulds are fully charged and is filled to about the level *m* whereupon the same level will be attained in the outer dozzles *i*.

The provision of such dozzles will effect 55 great economy in the production of electrically melted steel and high grade Siemens steel as it is unnecessary in these cases to discard any of the upper part of the ingot to dispose of deleterious non-metallic inclusions. With proper casting temperature 60 and speeds with such steels, ingots up to fourteen by fourteen inches cross sectional area may be cast without serious major segregation occurring.

65 In a modification of the method above de-

scribed and adapted for use when applied to certain qualities or grades of steel reference is directed to Figure 3 of the drawings.

In this modification there are applied to the upper ends of the outer moulds *h* the 70 stoppers *n* as of cast iron carried by rods or the like *o* having holes *p* at determined distances along same. The said stoppers, which as shown are almost equal in area to the cross section of the mould are held in a predetermined position in the mould by 75 passing a bar through one of the holes *p*, the bar seated on the top of the mould, or other means for adjustably positioning the stoppers may be used. The casting proceeds 80 down the central mould *g* until the metal in the outer moulds *h* has risen just into contact with the stoppers, whereupon said stoppers immediately cause the cast metal to freeze over and solidify at the surface. The 85 casting in the central mould is then continued at a reduced speed until the metal in the said central mould has attained a level several inches higher than the stoppered surface of the ingots in the outer moulds. Into 90 the central mould is then inserted a hot feeder head or "dozzle" *q* which is filled with metal, the object of the greater volume of metal in the central mould (at a higher level than the metal in the outer moulds) being to 95 eliminate contraction cavities within the ingots in the outer moulds. The method also actually effects the feeding of the outer ingots under pressure from the central ingot. The runner bricks *c* are preferably of larger 100 bore than previously specified for this method.

As aforesaid this modification in the casting method is applied to certain steels, whereas other steels will be provided with 105 hot feeder heads or "dozzles" for each ingot as referred to in the method described with reference to Fig. 1.

In Fig. 4 there is illustrated a further 110 modification somewhat different to that last described in that the stoppers *n* are replaced by a heated feeder head or "dozzle" *r* of the particular form shown having a recessed bottom and a central vent *v* from said cavity to the exterior. The same principle of feeding at the bottom from superimposed metal in the central mould is used as in the method described with reference to Fig. 3 but the hot feeder head renders the feeding more 115 certain. This feeder head is held in position in the outer mould *h* by means of a steel rod *s* loosely inserted into an aperture *t* in the head and a stopper *u* or other weight is placed on the head to prevent the head from floating up on the metal in the mould.

In the casting operation, when the metal 120 has filled the major cavity in the hot feeder head *r* the vent *v* is closed by means of the stopper *u* and casting into the central mould without stopping proceeds until a level sev- 125 130

eral inches above the line  $\alpha-\alpha$  is attained. An ordinary heated feeder head such as  $l$  (Fig. 1) is then inserted in the central mould and filled.

5 This method is of particular advantage when cast in the better grades of steel.

To now refer to the further form of stopper illustrated in Figs. 5 to 13, such a stopper as aforesaid is adapted for use when

10 producing large ingots. The frame of cast iron or cast steel is shown at  $A$  and  $A^1$  in Figs. 5 and 6 in plan view and section respectively and in similar views in Figs. 3, 7 and 8 at right angles to Figs. 5 and 6.

15 All these Figures 5 to 8 show the shape of frame designed to receive the bricks of silica or other refractory material shown in Figs. 10 to 13 and also indicate the provision of lugs  $F$   $F$  positioned on opposite sides of the

20 frame. Fig. 9 shows the stopper assembled for use,  $H$  designating the stopper rod provided with the series of holes  $H^2$  and pro-

25 vided with legs  $H^1$   $H^1$  which loosely fit the lugs  $F$   $F$  on the frame. In Figs. 10 and 11,  $D$   $D^1$  and  $E$   $E^1$  show the silica bricks provided with recesses  $D^2$  and  $E^2$  respectively.

Three or more of such bricks are used with each stopper to form a head substantially 30 hemispherical in shape below, and placed at the top of the ingot in the outer moulds. For the central mould, when making large ingots an ordinary feeder head may be used instead of a heater feeder head.

35 When making such large ingots the bore of the runner bricks will be increased in proportion to the size of the ingots to be produced so that the metal may flow from the central to the outer ingots during solidification.

40 In producing large ingots it would be impossible to manipulate heated feeder heads and it is therefore intended to use the composite stopper of steel and refractory material on the outer moulds and to have 45 metal superimposed in the central mould and an ordinary or brick lined head on said central mould.

Advantages of the methods described above are as follows:—

50 The weight of metal in the centre or feeder mould is always slightly in excess of the weight in any other mould of the group, whereby back-pressure is overcome and the metal rises evenly in each of the outer moulds

55 under the constant slight excess in the central mould. Liquid steel will, of course, find its own level in common with other liquids, but it is must be borne in mind that the metal in the outer moulds is cooler, more viscous, 60 and exerts more back pressure progressively as the filling of the moulds approaches completion. This is the outstanding defect of trumpet-casting that is to say, there comes a time (unless the metal is excessively hot)

65 when the cooling of the upper metal in the

moulds generates sufficient backpressure to prevent any hot metal entering the mould at the bottom. This often occurs and prevents the production of ingots of requisite weight: also it frequently occurs that ingots of uneven weight are produced from a "cluster" and this raises manifold difficulties of production.

The scrap produced by the improved method is less than that produced by trumpet casting as the metal remaining in the trumpet is always scrap.

The metal rises evenly and equally in all moulds notwithstanding that some may be placed further from the central mould than others. This is a function of balanced pressures which is absent when trumpet casting is used.

Costs are reduced as the expensive pipes and tundish for the trumpet are abolished. 85 The reduction of scrap is also a factor of costs.

Other advantages derived from the methods of the present invention are that casting may take place at a lower temperature, thereby conferring superior physical qualities upon steel; that the product of sound material from the ingots is very much greater than is the case with the present methods of ingot production; that the ingots 90 produced by the methods are free from surface and subcutaneous defects owing to the very even and regular rise of metal in the moulds, as compared with the surging, which almost invariably occurs in the moulds when trumpet casting is used: that, owing to the casting taking place at a lower temperature, the deleterious segregations are greatly minimized in the ingots and that as compared with the present system of casting, 95 particularly in the case of Tungsten steels, as well as to the electric, the Bessemer, and the open hearth products a steel of much greater homogeneity is obtained. By the adoption of this method by crucible steel 100 makers the incidental variations of composition due to the complex reactions in the crucible are averaged by the mixing of the contents of twelve or more crucibles in a ladle, and casting the whole of these simultaneously in a set of moulds.

What I claim as my invention and desire to secure by Letters Patent of the United States is:—

1. An apparatus for casting metal ingots 120 comprising a base plate having a central recess, channelled runner bricks radiating from said recess, a central mould disposed above said recess and outer moulds disposed above and communicating from below with 125 the outer ends of each of said runner bricks whereby the number of ingots produced is in accordance with the number of outer moulds plus that in the central mould, and metal stoppers adapted for insertion into the outer 130

moulds at predetermined distances and to substantially fill the cross sectional area of said moulds, said stoppers each comprising a metal frame and a plurality of sections of 5 bricks carried thereby, said brick sections being of refractory material and recessed on their under surfaces, the recesses when the sections are assembled in the frame forming a substantially hemispherical lower 10 surface.

2. An apparatus for casting metal ingots comprising a base plate having a central recess, channelled runner bricks radiating from said recess, a central mould disposed 15 above said recess and outer moulds disposed above and communicating from below with the outer ends of each of said runner bricks whereby the number of ingots produced is in accordance with the number of outer moulds 20 plus that in the central mould, and metal

25 stoppers adapted for insertion into the outer moulds at predetermined distances and to substantially fill the cross sectional area of said moulds, said stoppers each comprising a metal frame and bricks of refractory material carried thereby, lugs formed on the frame, a handle detachably connected to the lugs, said handle having vertically spaced perforations therein, and pins adapted for insertion through the perforations, said pins 30 engaging the upper surfaces of the moulds for limiting the distance of insertion of the stoppers.

In witness whereof I have signed this specification in the presence of two wit- 35 nesses.

GEO. BATTY.

Witnesses:

HENRY LECINBY COOPER,  
E. MABEL HODGKINSON.